

[54] REVERSAL MULTI-LAYER COLOR  
PHOTOGRAPHIC MATERIALS[75] Inventors: **Takeo Shimada; Yukio Yokota; Jun Hayashi**, all of Kanagawa, Japan[73] Assignee: **Fuji Photo Film Co., Ltd.**, Kanagawa, Japan[22] Filed: **Sept. 28, 1972**[21] Appl. No.: **293,276**

## [30] Foreign Application Priority Data

Sept. 30, 1971 Japan..... 46-76515

[52] U.S. Cl..... **96/22, 96/55, 96/74**[51] Int. Cl. .... **G03c 1/40, G03c 1/08, G03c 5/50**[58] Field of Search ..... **96/74, 55, 97, 22**

## [56] References Cited

## UNITED STATES PATENTS

2,688,539 9/1954 Heimbach et al..... 96/74 X

2,704,711 3/1955 Hanson, Jr..... 96/74 X

2,763,549 9/1956 Hanson, Jr..... 96/74 X

2,772,163 11/1956 Tong..... 96/97  
3,244,520 4/1966 Schulte et al..... 96/55

Primary Examiner—Ronald H. Smith

Assistant Examiner—Alfonso T. Suro Pico

Attorney, Agent, or Firm—Sughrue, Rothwell, Mion,  
Zinn and Macpeak

## [57] ABSTRACT

A reversal multi-layer color photographic light-sensitive material having on a support a red sensitive silver halide emulsion layer, a green sensitive silver halide emulsion layer, and a blue sensitive silver halide emulsion layer which is capable of forming after exposure upon development with color developing solutions containing a diffusible cyan coupler, a diffusible yellow coupler, and a diffusible magenta coupler, respectively, cyan, yellow, and magenta color images, in which the red sensitive silver halide emulsion layer of the color photographic material contains a diffusion resistant cyan coupler is disclosed.

15 Claims, No Drawings

## REVERSAL MULTI-LAYER COLOR PHOTOGRAPHIC MATERIALS

### BACKGROUND OF THE DISCLOSURE

#### 1. Field of the Invention

The present invention relates to a reversal multi-layer color photographic light-sensitive material and more particularly to a reversal multi-layer color photographic material showing less or substantially no color mixing from color developing solutions.

#### 2. Description of the Prior Art

As multi-layer color photographic light-sensitive materials each having on a support a red sensitive emulsion layer, a green sensitive emulsion layer, and a blue sensitive emulsion layer, there are generally two types: one containing in the photographic emulsion layers color formers (hereinafter called "couplers") capable of forming dyes by reaction with the oxidation product of a silver halide and an aromatic amino type developing agent and the other which does not contain couplers in the photographic emulsion layers.

Because the color photographic material of the type which does not contain couplers in the photographic emulsion layers is processed with color developing solutions containing couplers, it is superior in sharpness to the color photographic material of the type containing couplers in the photographic emulsion layers. However, in the conventional color photographic material of this type, undesirable dyes which should not be present are formed in a photographic emulsion layer together with the desired dye appropriate to that layer upon development to cause color mixing, and thus the color reproduction of the developed color photographic material is not good. For instance, when a reversal color photographic light-sensitive material having on a support a red sensitive emulsion layer, a green sensitive emulsion layer, and a blue sensitive emulsion layer each of which does not contain a coupler is after image exposure subjected to (successively) a black and white development, a cyan color development, a yellow color development, and a magenta color development (hereinafter, this is designated for brevity as "reversal color development" or "reversal color developing process,") a yellow dye and a magenta dye are formed in the red sensitive emulsion layer in addition to a cyan dye to form a slightly greenish or purplish cyan dye image, and thus a cyan color having high color purity is not obtained.

The cause of such color mixing is believed to be as follows: That is to say, when the above described reversal color photographic material of the type not containing couplers in the photographic emulsion layers is developed in the order described above, the red sensitive emulsion layer developed by a cyan color forming developing solution is further subjected to the subsequent yellow color development and magenta color development. Hence, if the development of the red sensitive emulsion layer has not been completely finished, the remaining development occurs in the red sensitive emulsion layer with the yellow color developing solution or the magenta color developing solution to cause a yellow color mixing or a magenta color mixing in the cyan image. In order to overcome such a difficulty, various methods have been proposed. For instance, a method is provided in which in order to conduct the cyan color development as quickly as possible a diffusible developing accelerator is incorporated in the cyan

color developing solution to complete the development of the red sensitive emulsion layer. This proposed method is an improvement in the developing solution. On the other hand, because the red sensitive emulsion layer of a color photographic material is the lowermost layer on the support thereof and thus the development of the red sensitive layer generally tends to be delayed in comparison with the developments of the blue sensitive layer or green sensitive layer caused by delay in the diffusion of the color developing solution, the addition of a developing accelerator to the red sensitive emulsion layer has also been proposed. However, such a technique is greatly limited since the addition of the developing promoter results in adverse influences on other important photographic properties of the color photographic light-sensitive material.

### SUMMARY OF THE INVENTION

An object of this invention is, therefore, to provide 20 a reversal color photographic light-sensitive material of the type which does not contain couplers in the photographic emulsion layers capable of forming upon reversal color development a cyan dye image having high color purity unaccompanied by yellow color mixing and magenta color mixing.

Another object of this invention is to provide a multi-layer color photographic light-sensitive material capable of forming a high color density upon reversal color development.

30 As the result of much research, it has been found that the above-described objects of this invention can be attained by incorporating a diffusion resistant cyan coupler in the red sensitive silver halide emulsion layer of a reversal color photographic light-sensitive material, preferably in an amount of from 0.0005 to 0.5 mol per mol of silver halide in the emulsion layer.

That is to say, it has astonishingly been found that a diffusion resistant cyan coupler contained to a very small extent in the red sensitive emulsion layer promotes cyan development in the cyan developing step to, thereby, prevent the silver halide in the red sensitive emulsion layer from remaining undeveloped after the cyan development and also to prevent the occurrence of yellow or magenta color mixing in the cyan image. 45 Such an astonishing advantage or effect has not been anticipated from the descriptions of known publications and the general common knowledge of production techniques for color photographic materials.

### 50 DETAILED DESCRIPTION OF THE INVENTION

In a multi-layer color photographic light-sensitive material wherein a red sensitive emulsion layer is positioned at the lowermost position on the support and a green sensitive emulsion layer and a blue sensitive emulsion layer are formed successively on the red sensitive layer, the development of the red sensitive layer tends to be delayed in comparison with other emulsion layers and further magenta color mixing and yellow color mixing tend to occur in the cyan dye image with conventional techniques. Where these points are considered, the advantage of the present invention will be highly appreciated.

60 The diffusion resistant cyan couplers used in this invention can be selected over a very wide range of compounds, for instance, compounds having from 15 to 44 carbon atoms can be selected from the generally known cyan couplers described in, e.g., W. Pelz, *Mit-*

teilungen aus den Forschungslaboratorien der Agfa, Le-  
verkusen, Munich; III 156-174(1961). The compounds  
represented by the general formula (I) or (II) give par-  
ticularly good results:



wherein R<sub>1</sub> and R<sub>2</sub> each represents a hydrogen atom, a straight chain or branched chain alkyl group having, preferably from 1 to 30 carbon atoms, such as methyl, ethyl, propyl, isopropyl, butyl, sec-butyl, tert-butyl, amyl, isoamyl, hexyl, octyl, decyl, dodecyl, pentadecyl, octadecyl, eicosyl, docosanyl, triacontanyl, etc. a cyclic alkyl group (such as a cyclohexyl group, a terpentyl group, and a norbornyl group), an aryl group (such as a phenyl group and a naphthyl group), a heterocyclic group (such as a benzimidazolyl group and benzthiazolyl group), or a non-metallic atomic group necessary for forming a heterocyclic ring (such as a morpholine ring and a piperidine ring) or R<sub>1</sub> and R<sub>2</sub> together can combine to form a heterocyclic group comprising non-metallic atoms; R<sub>5</sub> represents a hydrogen atom, an alkyl group, preferably having from 1 to 30 carbon atoms, an aryl group, a heterocyclic group, an amino group (such as an amino group, an alkylamino group, an arylamino group, and a heterocyclic amino group), a carbonamide group (such as an alkylcarbonamide group, an arylcarbonamide group, and a heterocyclic carbonamide group), a sulfonamide group (such as an alkylsulfonamide group, an arylsulfonamide group, and a heterocyclic sulfonamide group), a sulfamyl group (such as an alkylsulfamyl group, an arylsulfamyl group, and a heterocyclic sulfamyl group), a carbamyl group (such as an alkylcarbamyl group, an arylcarbamyl group, and a heterocyclic carbamyl group), or a ureido group (such as an N-alkylureido group and an N-arylureido group); R<sub>3</sub>, R<sub>4</sub>, R<sub>6</sub>, R<sub>7</sub> and R<sub>8</sub> each represents the groups as described above for R<sub>5</sub>, a halogen atom, or an alkoxy group, preferably having from 1 to 22 carbon atoms which may be substituted by a halogen atom, hydroxy group, amino group, carboxy group, alkoxy carbonyl group, alkylamide group, arylamide group, diacylamino group such as succinimide, alkoxy, aryloxy etc.; and X and Y each represents a hydrogen atom or a group capable of being split off at coupling, such as a halogen atom, a thiocyanato group, an acyloxy group, an alkoxy group, and an aryloxy group; in which X further represents a cyclic imide group (such as maleimide group, a succinimide group, a 1,2-dicarboxyimide group, and a phthalimide group).

At least one of R<sub>1</sub>, R<sub>2</sub>, R<sub>3</sub>, R<sub>4</sub>, R<sub>5</sub>, R<sub>6</sub>, R<sub>7</sub> and R<sub>8</sub> is advantageously further substituted by any of the ballasting groups well known in the art.

Each of the above described alkyl group, aryl group, and heterocyclic group represented by R<sub>1</sub> or R<sub>2</sub> may be substituted with a halogen atom, a nitro group, a hy-

droxyl group, a carbonyl group, an amino group (such as an amino group, an alkylamino group, a dialkylamino group, an anilino group, and an N-alkylanilino group), an aryl group, a carboxyester group (such as a carboalkoxy group and a carboallyloxy group), an amide group (such as an acetamide group, a butylamide group, an ethylsulfonamide group, an N-methylbenzamide group, an N-propylbenzamide group and a 4-t-butylbenzamide group), a carbamyl group (such as a carbamyl group, an N-octadecylcarbamyl group, an N,N-dihexylcarbamyl group, an N-methyl-N-phenylcarbamyl group, and a 3-pentadecylphenylcarbamyl group) a sulfamyl group (such as an N-propylsulfamyl group and an N-tolylsulfamyl group), an alkoxy group (such as an ethoxy group and an octadecyloxy group), an aryloxy group (such as a phenoxy group, a tolyloxy group, and a naphthoxy group), a sulfo group, a sulfonyl group (such as a methylsulfonyl group, an octadecylsulfonyl group, an ethoxysulfonyl group, a decoxysulfonyl group, a phenylsulfonyl group, a tolylsulfonyl group, and a phenoxy sulfonyl group), and the like.

Furthermore, each of the alkyl group, the aryl group, and the heterocyclic group represented by R<sub>5</sub> may also be substituted by the same groups as described in regard to the groups R<sub>1</sub> and R<sub>2</sub>.

Specific examples of the diffusion resistant cyan coupler which can be used in this invention are shown below although the diffusion resistant cyan couplers used in this invention are not to be interpreted as limited to them.

Coupler (1):



Coupler (2):



Coupler (3):



Coupler (4):



Coupler (5):



Coupler (6):



Coupler (7):



Coupler (8):



Coupler (9):



Coupler (10):



Coupler (11):



Coupler (12):



Coupler (13):



Coupler (14):



The diffusion resistant cyan couplers illustrated above may be prepared by well known methods. For instance, the production of the compound is illustrated in the U.S. Pat. Nos. 2,242,337; 2,324,832; 2,367,531; 5 2,357,395; and 2,474,293; in German Patent No. 1,036,053; and in British Patent specification No. 727,693.

The cyan coupler used in this invention may be incorporated in the photographic emulsion using well-known methods which are conventionally employed. For instance, cyan couplers having acid, e.g., carboxyl or sulfonic group may be incorporated into photographic emulsion as an aqueous alkaline solution thereof. As an alternative, cyan couplers not having 10 such acidic groups may be dissolved in an organic solvent such as described in U.S. Pat. No. 2,322,027, e.g. dibutyl phthalate and tricresyl phosphate, the solution is dispersed in an aqueous medium such as an aqueous solution of gelatin, and then the dispersion is added to the photographic emulsion (see, e.g., C. E. K. Mees and T. H. James; *The Theory of the Photographic Process*; 3rd Edition, published by Macmillan Co. 1966, page 393). Or, the cyan coupler can be melted by heating and the molten coupler directly dispersed in the emulsion or the aqueous medium.

The diffusion resistant cyan coupler may be incorporated in the photographic emulsion in any step before coating but it is desirable to incorporate it in a step between post-ripening and coating.

20 The amount of the diffusion resistant cyan coupler depends upon the nature of the silver halide photographic emulsion employed but in general ranges from 0.0005 to 0.5 mol per mol of the silver halide in the red sensitive emulsion layer, although the invention is not limited to this range. Furthermore, the diffusion resistant cyan couplers used in this invention may be used alone or used as a combination of two or more such couplers.

25 As the silver halide emulsion which can be employed 30 as the red sensitive emulsion layer, a gelatino silver iodobromide emulsion or a gelatino silver chloroiodobromide emulsion containing from 0.1 to 10 mol percent of iodide ion per mol of the silver halide is particularly preferred but other silver halide emulsions such as 35 a silver chloride emulsion, a silver chlorobromide emulsion, or a silver bromide emulsion can also be employed.

30 The silver halide photographic emulsion may have been chemically sensitized by method well known in 40 the art, e.g., by a labite sulfur containing compound, such as ammonium thiosulfate and allylthiocarbamide; a gold compound such as a complex salt of univalent gold and thiocyanic acid; a reducing agent such as stannous chloride; a polyalkylene oxide derivative; or a combination thereof. Also, the silver halide photographic emulsion may contain a stabilizer such as 4-hydroxy-6-methyl-1,3,3a,7-tetraazaindene, benzimidazole, and 1-phenyl-5-mercaptopotetrazole and a hardening agent such as formaldehyde or mucobromic acid. 45 Moreover, the photographic emulsion may contain a coating aid such as saponin or sodium alkylbenzenesulfonate.

50 As a sensitizing dye for providing the red sensitivity 55 to the silver halide photographic emulsion, a cyanine dye and a merocyanine dye capable of sensitizing the

emulsion in the wave length region of from 580 to 700  $\mu$  may be used alone or as combinations thereof.

It is desirable that the red sensitive photographic emulsion containing the diffusion resistant cyan coupler be first applied to a support and then a green sensitive emulsion layer, a yellow filter layer, and then a blue sensitive emulsion layer be formed thereon in this order. It is also desirable that the green sensitive emulsion layer and the blue sensitive emulsion layer contain no couplers but the green sensitive emulsion layer may contain a diffusion resistant magenta coupler and the blue sensitive emulsion layer may contain a diffusion resistant yellow coupler.

The reversal color photographic material having the red sensitive emulsion layer containing the diffusion resistant cyan coupler is desirably processed using the conventional reversal color photographic developing process.

Each of the cyan, magenta and yellow color developing solutions contains at least a color developing agent and a diffusible coupler capable of being colored cyan, magenta, and yellow, respectively.

Examples of color developing agents used in the color developing solutions are generally the well-known p-phenylenediamine derivatives such as 4-amino-N,N-diethylaniline, 4-amino-N,N-diethyl-3-methylaniline, 4-amino-3-methyl-N-methyl-N-( $\beta$ -methylsulfonamidoethyl)aniline, and 4-amino-3-methyl-N-ethyl-N-( $\beta$ -hydroxyethyl)aniline (see, e.g., C. E. K. Mees and T. H. James; *The Theory of the Photographic Process*; 3rd Edition, 387(1966), published by the Macmillan Co.).

Examples of the diffusible cyan coupler are the well-known phenolic couplers, such as 2-chloro-1-naphthol, 2,4-dichloro-1-naphthol, 1-hydroxy-N-butyl-2-naphthamide, 1-hydroxy-N-(2-acetamidophenethyl)-2-naphthamide, etc., (see, Mees et al., *supra*, page 387). Examples of the diffusible magenta couplers are open chain methylenic couplers such as acylacetone, 2-cyanoethylbenzofuran, and benzylacetone and cyclic methylenic couplers such as 1-phenyl-3-methyl-5-pyrazolone, 1-phenyl-3-(4-chlorobenzamide)-5-pyrazolone, 1-phenyl-3-(3-nitrobenzoylamino)-5-pyrazolone, 1-(2,4,6-trichlorophenyl)-3-(4-nitroanilino)-5-pyrazolone, etc. Also, examples of the diffusible yellow couplers are acylacetamide type open chain methylenic couplers such as 2-acetanilide, 2-aceto-2'-4'-dichloroacetanilide, 2-benzoylacetanilide, 2-benzoyl-2'-methoxyacetanilide, 2-benzoyl-(4'-p-toluene-sulfonamido)-acetanilide, etc., (see, G. H. Broun et al; *Journal of the American Chemical Society*; Vol. 79, 2,919-2,927(1957)).

The present invention will be further illustrated in greater detail by reference to the following examples. Unless otherwise indicated, all parts and percents are by weight.

#### EXAMPLE 1

A gelatino silver iodobromide emulsion for reversal color photography which had been subjected to sulfur sensitization and gold sensitization was melted by heating, sensitized for the red region, and the red sensitive silver halide emulsion thus prepared was divided into several portions. To each of the red sensitive emulsions was added an alkaline aqueous solution of the cyan coupler shown in Table 1 and then the pH of the emul-

sion was adjusted to 7.0 by adding citric acid. The red sensitive reversal color photographic emulsion containing the cyan coupler was applied to a cellulose triacetate film base so that the amount of silver was 15 mg/100 cm<sup>2</sup> and then a green sensitive reversal color photographic emulsion containing no magenta coupler, a coating composition for a yellow filter layer, and a blue sensitive reversal color photographic emulsion containing no yellow coupler were applied to the red sensitive emulsion layer in this order and dried.

The silver iodobromide emulsion for the red-sensitive layer contained 5 mole percent iodide. The emulsions for the green-sensitive and blue-sensitive layers were also silver iodobromide emulsions containing 5 mole percent iodide. The yellow filter layer contained yellow colloidal silver.

The samples of the reversal color photographic light-sensitive materials thus prepared were subjected to overall cyan exposure using an NSG II-type actinometer and then subjected to the following reversal color photographic processings:

|     |                              |      |        |
|-----|------------------------------|------|--------|
| 1.  | Pre-hardening                | 27°C | 1 min. |
| 2.  | Water Washing                | do.  | do.    |
| 3.  | Negative Development         | do.  | 4 min. |
| 4.  | Water Washing                | do.  | 3 do.  |
| 5.  | Reversal Red Flash Exposure  |      |        |
| 6.  | Cyan Color Development       | 27°C | 5 min. |
| 7.  | Water Washing                | do.  | 2 do.  |
| 8.  | Reversal Blue Flash Exposure |      |        |
| 9.  | Yellow Color Development     | do.  | 5 min. |
| 10. | Water Washing                | do.  | 2 do.  |
| 11. | Reversal White Exposure      |      |        |
| 12. | Magenta Color Development    | 27°C | 5 min. |
| 13. | Water Washing                | do.  | 2 do.  |
| 14. | Silver Bleaching             | do.  | 5 do.  |
| 15. | Fixing                       | do.  | 3 do.  |
| 16. | Water Washing and Drying     |      |        |

The compositions of the processing baths used in the above processings were as follows:

|    |                                                 |         |  |
|----|-------------------------------------------------|---------|--|
| 40 | Prehardening Solution:                          |         |  |
|    | Concentrated Sulfuric Acid                      | 1.7 cc  |  |
|    | Borax (10-hydrate)                              | 20 g    |  |
|    | Potassium Bromide                               | 2.3 g   |  |
|    | Sodium Sulfate                                  | 200 g   |  |
|    | 37% Formaldehyde                                | 10 cc   |  |
|    | Sodium Bisulfite                                | 1 g     |  |
|    | Water added to make 1000 cc.                    |         |  |
| 45 | Negative Developing Solution:                   |         |  |
|    | N-Methyl-p-aminophenol Sulfate                  | 5 g     |  |
|    | Anhydrous Sodium Sulfite                        | 79 g    |  |
|    | Hydroquinone                                    | 2 g     |  |
|    | Sodium Carbonate (monohydrate)                  | 40 g    |  |
|    | Potassium Bromide                               | 3.5 g   |  |
|    | Potassium Thiocyanate                           | 2.0 g   |  |
|    | 0.1% Potassium Iodide                           | 12.5 cc |  |
|    | Sodium Hydroxide                                | 1.0 g   |  |
|    | Water added to make 1000 cc.                    |         |  |
| 50 | Cyan Color Developing Solution:                 |         |  |
|    | Potassium Bromide                               | 2.0 g   |  |
|    | 0.1% Potassium Iodide                           | 20 cc   |  |
|    | Potassium Thiocyanate                           | 3.0 g   |  |
|    | Anhydrous Sodium Sulfite                        | 10 g    |  |
|    | Sodium Carbonate (monohydrate)                  | 30 g    |  |
|    | Sodium Hydroxide                                | 2.0 g   |  |
|    | 5-Nitrobenzimidazole Nitrate                    | 0.5 g   |  |
|    | 2,4-Dichloro-1-naphthol                         | 2.0 g   |  |
|    | 4-Amino-3-methyl-N,N-diethylaniline             |         |  |
|    | Hydrochloride                                   | 3.0 g   |  |
|    | Water added to make 1000 cc.                    |         |  |
| 60 | Yellow Color Developing Solution:               |         |  |
|    | Sodium Sulfite                                  | 5.0 g   |  |
|    | N,N-Diethyl-p-phenylenediamine                  |         |  |
|    | Hydrochloride                                   | 1.2 g   |  |
|    | Sodium Carbonate (monohydrate)                  | 20.0 g  |  |
|    | Potassium Bromide                               | 0.3 g   |  |
|    | 0.1% Potassium Iodide                           | 2.0 cc  |  |
|    | 2-Benzoyl-(4'-p-toluenesulfonamide)-acetanilide | 1.0 g   |  |
|    | Sodium Hydroxide                                | 4.0 g   |  |
|    | Water added to make 1000 cc.                    |         |  |

Continued

|                                     |       |
|-------------------------------------|-------|
| Magenta Color Developing Solution:  |       |
| Sodium Sulfite                      | 5.0 g |
| 4-Amino-3-methyl-N,N-diethylaniline |       |
| Hydrochloride                       | 2.0 g |
| Potassium Bromide                   | 0.2 g |
| 1-Phenyl-3-(3-nitrobenzoylamino)-   |       |
| 5-pyrazolone                        | 1.4 g |
| Sodium Hydroxide                    | 2.5 g |
| n-Butylamine                        | 5 cc  |
| Water added to make 1000 cc.        |       |
| Silver Bleaching Solution:          |       |
| Ferricyanide                        | 60 g  |
| Potassium Bromide                   | 20 g  |
| Water added to make 1000 cc.        |       |
| Fixing Solution:                    |       |
| Sodium Thiosulfate                  | 100 g |
| Sodium Sulfite                      | 15 g  |
| Water added to make 1000 cc.        |       |

Thereafter, the densities of the cyan dye image thus obtained were measured using a green filter and a red filter, respectively, the results of which are shown in the following table.

Table 1

| Cyan Coupler | Amount * | Cyan Density | Yellow Density | Magenta Density |
|--------------|----------|--------------|----------------|-----------------|
| None         | —        | 1.85         | 0.75           | 0.53            |
| Coupler (1)  | 0.005    | 1.91         | 0.73           | 0.53            |
| do.          | 0.02     | 2.12         | 0.69           | 0.52            |
| Coupler (2)  | 0.005    | 1.88         | 0.74           | 0.52            |
| do.          | 0.02     | 2.05         | 0.70           | 0.50            |
| Coupler (3)  | 0.005    | 1.90         | 0.73           | 0.53            |
| do.          | 0.02     | 2.11         | 0.70           | 0.49            |
| Coupler (4)  | 0.005    | 1.88         | 0.74           | 0.52            |
| do.          | 0.02     | 2.07         | 0.71           | 0.50            |
| Coupler (5)  | 0.005    | 2.00         | 0.70           | 0.50            |
| do.          | 0.02     | 2.18         | 0.65           | 0.47            |
| Coupler (6)  | 0.005    | 1.93         | 0.72           | 0.50            |
| do.          | 0.02     | 2.08         | 0.69           | 0.48            |
| Coupler (7)  | 0.005    | 1.95         | 0.72           | 0.52            |
| do.          | 0.02     | 2.15         | 0.67           | 0.47            |

\* mol/mol AgX (AgX denotes silver halide).

As is clear from the results contained in Table 1 above, the density of the cyan color was increased and the density of magenta and yellow colors were decreased by the addition of the diffusion resistant cyan couplers in comparison with the control case containing no such diffusion resistant cyan coupler. This demonstrates that the magenta mixing and yellow mixing were reduced and the cyan density was increased by the application of this invention.

### EXAMPLE 2

The red sensitive silver iodobromide emulsion for reversal color photography as employed in Example 1 was melted by heating and divided into several portions. 5 g of the diffusion resistant cyan coupler shown in Table 2 was dissolved in a mixture of 10 g of tricresyl phosphate and 20 g of ethyl acetate, the solution was dispersed in 50 g of aqueous gelatin solution together with a dispersion assistant (sodium dodecyl benzene sulfonate), and the coupler dispersion obtained was added to the above-described photographic emulsion prepared above in an amount as shown in Table 3. Then, the pH of the photographic emulsion was adjusted to 7.0.

The red sensitive reversal color photographic emulsion containing the diffusion resistant cyan coupler was applied to a cellulose triacetate film base so that the amount of silver was 15 mg/100 cm<sup>2</sup> and then a green sensitive reversal color photographic emulsion containing no magenta coupler, a coating composition for a

yellow filter layer, and a blue sensitive reversal color photographic emulsion containing no yellow coupler in order were applied to the red sensitive layer and dried as in Example 1. These layers are the same as those used in Example 1 except the yellow filter layer contains a yellow dye.

The samples thus prepared were exposed in the same way as described in Example 1, developed, and the densities of the cyan image thus formed were measured. The results obtained are shown in Table 2.

Table 2

|    | Cyan Coupler | Amount * | Cyan Density | Yellow Density | Magenta Density |
|----|--------------|----------|--------------|----------------|-----------------|
| 15 | None         | —        | 1.85         | 0.75           | 0.53            |
|    | Coupler (7)  | 20       | 1.87         | 0.73           | 0.50            |
|    | do.          | 100      | 2.10         | 0.70           | 0.48            |
|    | Coupler (8)  | 20       | 1.89         | 0.72           | 0.51            |
|    | do.          | 100      | 2.08         | 0.70           | 0.48            |
|    | Coupler (9)  | 20       | 1.87         | 0.72           | 0.51            |
|    | do.          | 100      | 2.12         | 0.69           | 0.49            |
|    | Coupler (10) | 20       | 1.90         | 0.70           | 0.50            |
|    | do.          | 100      | 2.17         | 0.65           | 0.45            |
|    | Coupler (11) | 20       | 1.88         | 0.72           | 0.51            |
|    | do.          | 100      | 2.08         | 0.70           | 0.48            |
|    | Coupler (12) | 20       | 1.87         | 0.73           | 0.50            |
|    | do.          | 100      | 2.10         | 0.70           | 0.47            |
|    | Coupler (13) | 20       | 1.90         | 0.71           | 0.49            |
|    | do.          | 100      | 2.15         | 0.66           | 0.44            |
|    | Coupler (14) | 20       | 1.88         | 0.73           | 0.51            |
|    | do.          | 100      | 2.08         | 0.70           | 0.48            |

\* The amount of the coupler dispersion in g/mol AgX.

30 As is shown by the results contained in the above table, the cyan density was increased and the magenta and yellow densities were decreased by the addition of the cyan couplers according to the present invention.

35

### EXAMPLE 3

40 The samples of color photographic light-sensitive materials were prepared by coating the silver halide photographic emulsions described in Example 1 to a film base and dried in the same manner as described in Example 1 except that the diffusion resistant cyan coupler shown in Table 1 was used in each sample and the hardening process was conducted for 3 minutes at 27°C in a hardening bath having the following composition.

|    | Pre-hardening Solution:              |         |
|----|--------------------------------------|---------|
| 50 | Water                                | 800 cc  |
|    | Dimethoxytetrahydrofuran             | 4.3 cc  |
|    | 0.8 N H <sub>2</sub> SO <sub>4</sub> | 5.41 cc |
|    | Sodium p-Toluenesulfonate            | 0.5 g   |
|    | Sodium Sulfate                       | 153 g   |
|    | Potassium Acetate                    | 2.3 g   |
|    | Sodium Acetate                       | 20 g    |
|    | 37% Formalin                         | 27 cc   |

55 After the processings, the densities of the cyan dye image were measured as described in Example 1, the results of which are shown in Table 3.

Table 3

|    | Cyan Coupler | Amount mol/mol AgX | Cyan Density | Yellow Density | Magenta Density |
|----|--------------|--------------------|--------------|----------------|-----------------|
| 65 | None         | —                  | 1.76         | 0.67           | 0.45            |
|    | Coupler (1)  | 0.0005             | 1.79         | 0.66           | 0.43            |
|    | do.          | 0.005              | 1.85         | 0.63           | 0.41            |
|    | do.          | 0.05               | 1.88         | 0.61           | 0.39            |
|    | do.          | 0.25               | 1.89         | 0.59           | 0.39            |

As is shown by the results contained in the above table, the cyan density was increased and the yellow and magenta densities were decreased by the addition of the cyan coupler.

## EXAMPLE 4

The gelatino silver iodobromide red sensitive emulsion for reversal color photography as used in Example 1 was melted by heating, an aqueous alkaline solution of Coupler (5) was added to the melt in an amount of 0.01 mol per mol of the silver halide and the pH of the mixture was adjusted to 7.0.

As described in Example 1, the red sensitive silver halide emulsion containing the diffusion resistant cyan coupler, the green sensitive emulsion containing no magenta coupler, a coating composition for yellow filter, and the blue sensitive emulsion containing no yellow coupler were applied to a cellulose triacetate film and dried.

The samples thus prepared were exposed and processed in the same manner as described in Example 1 except that different diffusible couplers from those of Example 1 were used in the cyan, yellow, and magenta color developing solutions and then the densities of the cyan images were measured.

The combinations of the diffusible couplers used in this example and the results of the reversal color developing procedures obtained are shown in Table 4. The numerical values in Table 4 are the difference in the yellow density, the difference in the cyan density, and the difference in the magenta density of the cyan images obtained in adding the diffusion resistant cyan coupler to the red sensitive silver halide emulsion layer and in not adding such a diffusion resistant cyan coupler to the red sensitive emulsion layer. The sign (+) shows that the density increased by the addition of the diffusion resistant cyan coupler to the red sensitive emulsion layer, while the sign (-) shows that the density decreased.

Thus, by the application of this invention, the cyan density was increased and the yellow and magenta densities were decreased in the case of conducting reversal color developing procedures with the color developing solution containing a diffusible coupler shown in Table 4 as compared with the case of not adding a diffusion resistant cyan coupler to the red sensitive emulsion layer.

Furthermore, when other diffusion resistant cyan couplers other than those employed in Examples 1, 2, 3, and 4 were used, essentially the same results were obtained. Also, in other reversal color photographic processings using processing baths having different

compositions than those of the above examples, essentially the same good results were obtained.

While the invention has been described in detail and in terms of specific embodiments thereof, it will be apparent that various changes and modifications can be made therein without departing from the spirit and scope thereof.

What is claimed is:

1. In a multi-layer reversal color photographic material having on a support a red sensitive silver halide emulsion layer, a green sensitive silver halide emulsion layer, and a blue sensitive silver halide emulsion layer capable of forming after exposure and black and white negative development cyan, yellow, and magenta dyed images respectively by the developments in three color developing solutions containing a diffusible cyan coupler, a diffusible yellow coupler, and a diffusible magenta coupler, respectively, the improvement comprising said red sensitive silver halide emulsion containing a diffusion resistant cyan coupler present in said red sensitive emulsion layer in an amount ranging from 0.005 to 0.5 mol per mol of the silver halide in said red sensitive emulsion layer wherein said blue-sensitive and said green-sensitive layers contain no color couplers after "layer" at the last line.

2. The multi-layer reversal color photographic material as set forth in claim 1, wherein said diffusion resisting cyan coupler is a compound represented by the formula

30

35



40 wherein R<sub>1</sub> and R<sub>2</sub> each represents a hydrogen atom, a straight chain alkyl group, a branched chain alkyl group, a cyclic alkyl group, an aryl group, a heterocyclic group, or a non-metallic atomic group necessary for forming a heterocyclic group; R<sub>3</sub> and R<sub>4</sub> each represents a hydrogen atom, a halogen atom, an alkyl group, an alkoxy group, an aryl group, a heterocyclic group, an amino group, a carbonamide group, a sulfonamide group, a sulfamyl group, a carbamyl group, or a ureido group; and X represents a hydrogen atom, a group capable of being split off at coupling, or a cyclic imide group.

Table 4

| Ex. No. | Cyan Coupler<br>(g/liter)                                          | Diffusible Coupler<br>Yellow Coupler<br>(g/liter) | Magenta Coupler<br>(g/liter)                                                                                 | Density Difference |                   |                    |
|---------|--------------------------------------------------------------------|---------------------------------------------------|--------------------------------------------------------------------------------------------------------------|--------------------|-------------------|--------------------|
|         |                                                                    |                                                   |                                                                                                              | Cyan<br>Density    | Yellow<br>Density | Magenta<br>Density |
| 1       | 2,4-Dichloro-1-naphthol (2 g/l.)                                   | 2-Benzoylaceto-anilide (1.8 g/l.)                 | 1-Phenyl-3-(4-chlorobenzamido)-5-pyrazolone (1.7 g/l.)<br>do.                                                | +0.20              | -0.07             | -0.05              |
| 2       | 1-Hydroxy-N-butyl-2-naphthamide (2 g/l.)                           | 2-Aceto-2',4'-dichloroaceto-anilide (1.8 g/l.)    | 2-Benzoyl-2-methoxyacetanilide (1.5 g/l.)                                                                    | +0.18              | -0.06             | -0.04              |
| 3       | 1-Hydroxy-N-(2-acetamidophenethyl)-2-naphthamide (1.8 g/l.)<br>do. | 2-Benzoyl-2-methoxyacetanilide (1.5 g/l.)         | 1-(2,4,6-Trichlorophenyl)-3-(4-nitroanilino)-5-pyrazolone (1.7 g/l.)<br>2-(Cyanocetyl)-benzofuran (1.5 g/l.) | +0.22              | -0.09             | -0.05              |
| 4       | do.                                                                | 2-Acetanilide (1.3 g/l.)                          | do.                                                                                                          | +0.18              | -0.06             | -0.04              |

3. The multi-layer color reversal photographic material as set forth in claim 1, wherein said diffusion resistant cyan coupler is a compound represented by the formula:



wherein R<sub>5</sub> represents a hydrogen atom, an alkyl group, an aryl group, a heterocyclic group, an amino group, a carbonamide group, a sulfonamide group, a sulfamyl group, a carbamyl group, or a ureido group; R<sub>6</sub>, R<sub>7</sub>, and R<sub>8</sub> each represents a hydrogen atom, a halogen atom, an alkyl group, an alkoxy group, an aryl group, a heterocyclic group, an amino group, a carbonamide group, a sulfonamide group, a sulfamyl group, a carbamyl group, or a ureido group; and Y represents a hydrogen atom or a group capable of being split off at coupling.

4. The multi-layer color reversal photographic material as set forth in claim 1, wherein said silver halide emulsion layer is silver iodobromide or silver chloroiodobromide containing from 0.1 to 10 mol percent of iodide per mol of silver halide.

5. The multi-layer color reversal photographic material as set forth in claim 1, wherein said diffusion resistant cyan coupler is

Coupler (1):



Coupler (2):



Coupler (3):



Coupler (4):



Coupler (5):



Coupler (6):



Coupler (7):



Coupler (8):



Coupler (9):



Coupler (10):



Coupler (11):



Coupler (12):



Coupler (13):



Coupler (14):



6. The multi-layer color reversal photographic material as set forth in Claim 1, wherein said red sensitive silver halide emulsion layer contains chemically sensitized silver halide.

7. The multi-layer color reversal photographic material as set forth in claim 1, wherein said silver halide in each of said emulsion layers is chemically sensitized.

8. In a process for forming color photographic images comprising image exposing a multi-layer reversal color photographic material including a support carrying a red sensitive silver halide emulsion layer, a green sensitive silver halide emulsion layer and a blue sensitive silver halide emulsion layer; developing said photographic material with a black and white developing solution and then subjecting said photographic material to color development with three color developing solutions, each containing a diffusible cyan coupler, a diffusible yellow coupler or a diffusible magenta coupler to form cyan, yellow and magenta dye images, respectively, the improvement which comprises reducing color mixing by including 0.005 to 0.5 mol of diffusion resistant cyan coupler per mol of silver halide in said red sensitive emulsion layer.

9. The process of claim 8 wherein said diffusion resisting cyan coupler is a compound represented by the formula



wherein R<sub>1</sub> and R<sub>2</sub> each represents a hydrogen atom, a straight chain alkyl group, a branched chain alkyl group, a cyclic alkyl group, an aryl group, a heterocyclic group, or a non-metallic atomic group necessary for forming a heterocyclic group; R<sub>3</sub> and R<sub>4</sub> each represents a hydrogen atom, a halogen atom, an alkyl group, an alkoxy group, an aryl group, a heterocyclic group, an amino group, a carbonamide group, a sulfonamide group, a sulfamyl group, a carbamyl group, or a ureido group; and X represents a hydrogen atom, a group capable of being split off at coupling, or a cyclic imide group.

10. The process of claim 8 wherein the diffusion resisting cyan coupler is a compound represented by the formula



wherein R<sub>5</sub> represents a hydrogen atom, an alkyl group, an aryl group, a heterocyclic group, an amino group, a carbonamide group, a sulfonamide group, a sulfamyl group, a carbamyl group, or a ureido group; R<sub>6</sub>, R<sub>7</sub>, and R<sub>8</sub> each represents a hydrogen atom, a halogen atom, an alkyl group, an alkoxy group, an aryl group, a heterocyclic group, an amino group, a carbonamide group, a sulfonamide group, a sulfamyl group, a carbamyl group, or a ureido group; and Y represents a hydrogen atom or a group capable of being split off at coupling.

11. The process of claim 8 wherein there is used as the silver halide in said red sensitive silver halide emulsion layer silver iodobromide or silver chloroiodobromide containing from 0.1 to 10 mol percent of iodide per mol of silver halide.

12. The process of claim 8 wherein said diffusion resisting cyan coupler is

10

Coupler (1):



15

Coupler (2):



20

Coupler (3):



30

Coupler (4):



35

Coupler (5):



40

Coupler (6):



45

Coupler (7):



50

Coupler (8):



55

Coupler (9):



Coupler (10):



Coupler (11):



Coupler (12):



Coupler (13):



Coupler (14):



15

20

13. The process of claim 8 wherein chemically sensitized silver halide is present in said red sensitive silver halide emulsion layer.

14. The process of claim 8 wherein said silver halide 25 in each of said emulsion layers is chemically sensitized.

15. The process of claim 8 wherein the blue sensitive silver halide emulsion and the green sensitive silver halide emulsion layer do not contain color couplers.

30

\* \* \* \* \*

35

40

45

50

55

60

65